

1

2,776,932

## PROCESS FOR OXIDIZING ASPHALTS

Harley F. Hardman, Lyndhurst, Ohio, assignor to The Standard Oil Company, Cleveland, Ohio, a corporation of Ohio

No Drawing. Application May 6, 1953,  
Serial No. 353,448

4 Claims. (Cl. 196—74)

This invention relates to an improved process for the treatment of asphalt stocks and more particularly to a process for producing asphalt having improved properties.

With the development of the extensive use of asphalt in bituminous type pavements, asphalts have been extensively investigated and a number of specifications have developed over the years. As more information has been accumulated, additional specifications have been added from time to time. However, penetration measurements, especially where made at different temperatures, are one of the most important characterizations, and penetration is invariably included in asphalt specifications.

Penetration is the consistency of a bituminous material, that is, the resistivity to deformation, and is expressed as the distance that a standard needle vertically penetrates a sample of the material under known conditions of loading, time and temperature. The test is standard in the industry. High penetrations indicate a softer asphalt.

Temperatures susceptibility is a calculated value and is a comparison of the consistency or hardness of the asphalt at some elevated temperature with the same property at a lower temperature. Numerically, it is the ratio of the penetration value of the asphalt measured at a higher temperature to the penetration of the asphalt at a lower temperature. Several different higher temperatures and several different lower temperatures have been proposed as the best for comparison purposes. For purposes of the present disclosure, the two values are taken at 77° F. and 32° F., respectively. The temperature susceptibility is therefore defined herein as the ratio of the penetration at 77° F. divided by the penetration at 32° F. The lower this number the more desirable is the asphalt. This stems from the fact that the asphalt must meet a rigid 77° F. penetration, and if it has a low temperature susceptibility it does not become as hard or brittle at low temperatures, and there is less tendency for pavements made with such asphalts to deteriorate under the stress of use at low temperatures.

In order to understand more fully the significance of the above specification, it is believed desirable to explain briefly the manner in which asphalt is made and the effect that the manufacturing procedures and the constitution of the asphalt may be expected to have upon the above-described specification.

When whole crude oil is distilled to remove all of the fractions that are volatile at atmospheric pressure up to a temperature below cracking, the undistilled remainder is commonly known as "reduced crude." This reduced crude is then subjected to further distillation and fractionation under a vacuum, and various volatile fractions comprising lubricating oil fractions, waxes, and cylinder stocks are removed overhead. This operation is often carried out in a fractionating column known as a

2

pipe still, and the petroleum residuum is often referred to as pipe still bottoms. The composition of the pipe still bottoms will vary somewhat depending upon the source of the crude oil and the extent to which the 5 volatile fractions were removed as overhead distillate. The pipe still bottoms as such are included with the term "asphaltic stock" as used herein and may be the final asphalt material or it may be further modified to form the final asphalt as explained herein.

10 Asphaltic stocks may be divided into two fractions, termed "petrolenes" and "asphaltenes." The petrolenes constitute the fraction which is soluble in 50 volumes of normal pentane, and the asphaltenes comprise the fraction which is insoluble in normal pentane. These 15 asphaltic stocks may be considered to be colloidal systems in which the asphaltenes constitute the dispersed phase and the petrolenes the dispersive phase. Since the petrolenes are generally liquids (although in some instances they have very high viscosities), and the asphaltenes are generally solids, the petrolenes may be regarded as plasticizers for the asphaltenes. The properties of the asphalt will be determined to some extent by the relative proportions of the asphaltenes and petrolenes. 20 The higher the proportion of the latter, the softer will be the asphalt. It will be obvious in view of this explanation that the larger the amount of petrolene fraction that is distilled overhead in the pipe still fractionation, the smaller will be the amount of petrolenes remaining in the residuum. It is possible to operate the 25 pipe still fractionation in such a way that no more than the requisite amount of petrolenes remains in the residuum to provide a "straight-run" asphalt of the desired penetration. For example, the pipe still may be operated under such conditions and for such a time that the residuum has a penetration of 70-80 at 77° F., a value commonly specified for asphalts.

In addition to the relative amounts of the petrolenes and asphaltenes, another factor that affects the properties of the asphalt is the character of the asphaltene 40 and petrolene fractions. The viscosity of the petrolene fraction may vary, and it will be obvious that the viscosity of this fraction will have an effect upon its plasticizing action and be instrumental in determination of the properties of the asphalt. Similarly the molecular weight 45 of the asphaltenes can vary and will affect the properties of the asphalt.

As the distillation in the pipe still is continued, it will be obvious that the more volatile petrolenes, i. e., those having lower viscosities, will be distilled overhead. 50 The petrolenes which remain are those of higher viscosities. Thus a straight-run asphalt will have petrolenes of a relatively higher viscosity.

The viscosity of the petrolenes is believed to be an 55 important characteristic of asphalt due to the effect thereon of ductility, softening point, bleeding tendency, low temperature brittleness, oxidation resistance, and stripping resistance. Petrolenes of low viscosity are particularly desirable in an asphalt to impart the last three properties. For this reason the straight-run asphalt is deficient in this respect.

Generally, however, the pipe still is not operated in a manner to produce a straight-run asphalt. Usually the residuum contains an amount of petrolenes in excess of 65 that to give an asphalt of the desired properties. Accordingly, it is common to heat the residuum alone or in the presence of a catalyst or accompanied by air blowing alone or in the presence of a catalyst to convert a portion of the petrolenes into asphaltenes.

The oxidation of the residuum, which is a commonly employed mode of operation, is usually effected by blowing air through the residue at a temperature of about 400

to 500° F. at a rate of about 30 to 50 cubic feet per minute per ton of asphalt charge until the desired penetration is obtained.

In accordance with the present invention, it has been found that the addition of certain catalysts to asphalts, before heating and before blowing if the asphalt is blown, produces a final asphalt product having an improved temperature susceptibility. The catalysts also result in hardening of the asphalt during the addition of the catalyst and before any oxidation or blowing is effected. With some stocks no oxidation or blowing is necessary, and with others the oxidation time is shortened.

In accordance with the invention, the asphalt derives its decrease in penetration from an increase both in the molecular weight of the asphaltenes and in their concentration in the asphalt. The asphalts treated or prepared in accordance with the invention possess a better temperature susceptibility than do straight-run asphalts or asphalts prepared by heating or air blowing without our catalysts.

As will be seen from the data hereinafter, the use of the catalysts of the invention, while permitting the usual conversion of petroleos to asphaltenes, causes a decrease in the viscosity of the petroleos. Apparently the heavier petroleos are selectively converted to asphaltenes by the use of our catalysts with the result that the petroline content has a lower viscosity with the consequent improvement in temperature susceptibility and low temperature brittleness. The use of the catalysts also causes an increase in asphaltene molecular weight as well as asphaltene content. This tends to produce a more complex asphaltene system which imparts the desirable low temperature susceptibility.

The catalysts employed in the process of the invention are the heavy metal fluoborates. The heavy metals may be any of those having an atomic number in excess of 22 and having a pronounced metallic character as distinguished from arsenic, for example, which is a metal having certain properties of an acid. Among the above mentioned heavy metals which may be employed are: vanadium, chromium, manganese, iron, cobalt, nickel, copper, zinc, molybdenum, cadmium, tin, antimony, tungsten, silver, lead and bismuth.

The catalysts are added to the asphalt stocks in quantities of about 0.1 to 5% by weight and preferably 1 to 3% by weight of the asphalt stock. The temperature of the asphalt during incorporation of the catalyst is not critical, but the asphaltic stock is heated or heated and blown with air until the requisite penetration is achieved, depending on the specifications to be met and the use to which the asphalt is to be put. Generally the temperature of the heating and/or heating and blowing is 200 to 500° F. for a few minutes to several days. The lower the temperature, the longer the time, and vice versa. Neither is critical as long as the desired final penetration is met.

The invention will be further illustrated by reference to the following specific examples.

The results of a series of tests are summarized in Tables I and II below. In preparing these samples, two different pipe still bottoms fractions were heated to 200 to 300° F., after which the catalyst was added and the mixture was held at this temperature until any visible evidence of reaction disappeared. The penetration was then measured to determine the amount of further oxidation necessary to obtain a satisfactory product. After measuring the penetration, the mixtures containing catalyst were heated to 425-450° F. and oxidized for a period sufficient to obtain a penetration of 70 to 80. Blank samples not containing the catalyst were also oxidized at 425 to 450° F. for the purpose of comparison. In each case the catalyzed asphalts had a lower temperature susceptibility than in the blank, i. e., the 100° F. pen. was lower and the 32° F. pen. was higher, from which it will be seen that the asphalt was stiffer at the higher temperature and softer at the lower temperature than was the blank. Tables I and II illustrate the temperature sus-

ceptibilities of the samples with various penetrations and show that the catalyzed asphalts were improved.

TABLE I

| Example | Catalyst         | Penetration |     |     | Soft. Pt. | Pen. 77°/Pen. 32° |
|---------|------------------|-------------|-----|-----|-----------|-------------------|
|         |                  | 100°        | 77° | 32° |           |                   |
| 10      | None             | 212         | 70  | 23  | 125       | 3.05              |
|         | 3% Cd fluoborate | 202         | 78  | 31  | 132       | 2.53              |
|         | 3% Fe fluoborate | 127         | 63  | 27  | 152       | 2.34              |
|         | 3% Ni fluoborate | 229         | 76  | 30  | 127       | 2.54              |
|         | 3% Pb fluoborate | 227         | 78  | 31  | 132       | 2.63              |
|         | 3% Zn fluoborate | 128         | 74  | 27  | 129       | 2.75              |

TABLE II

| Example | Catalyst                      | Penetration |     |     | Soft. Pt. | Pen. 77°/Pen. 32° |
|---------|-------------------------------|-------------|-----|-----|-----------|-------------------|
|         |                               | 100°        | 77° | 32° |           |                   |
| 20      | None                          | 226         | 78  | 23  | 113       | 3.39              |
|         | 3% Sn fluoborate <sup>1</sup> | 230         | 78  | 24  | 120       | 3.25              |

<sup>1</sup> The sample prepared with stannous fluoborate did not require any oxidation.

Data was also obtained showing the beneficial effects of the catalysts on the petroline viscosity and the asphaltene molecular weight of two different asphalt samples. These data are summarized in Table III.

TABLE III  
*Effect of catalysts on molecular weight and asphalt composition variables*

| Example | Catalyst                             | Petroleum, Vis. at 77° F. |        | Asphaltene, Mol. Wt. |
|---------|--------------------------------------|---------------------------|--------|----------------------|
|         |                                      | 100°                      | 77°    |                      |
| 35      | None                                 | 17,600                    | 12,260 | 2,610                |
|         | 3% Sn(BF <sub>4</sub> ) <sub>2</sub> | 5,210                     | 3,790  | 2,700                |
| 40      | None                                 | 17,600                    | 12,260 | 3,350                |
|         | 3% Fe(BF <sub>4</sub> ) <sub>2</sub> | 5,210                     | 3,790  | 4,385                |

By comparison with the corresponding blank, it is seen that the catalysts caused a decrease in petroline viscosity and an increase in asphaltene molecular weight, the change being greater the more effective the catalyst.

A reasonable interpretation of these data is that the fluoborate catalyst alters the oxidation of the petroleos to preferentially oxidize the heavier petroleos to asphaltenes, leaving the lighter petroleos in the asphalt to exert a better plasticizing action at lower temperatures. It is believed that the reduction in temperature susceptibility which is in effect a lowering of the point at which the asphalt becomes brittle is achieved by the presence of a petroline fraction which has a lower viscosity at lower temperatures. In other words, at low temperatures the petroleos are sufficiently fluid to exert a plasticizing action on the asphaltenes.

It will be obvious to those skilled in the art that many modifications may be made within the scope of the present invention without departing from the spirit thereof and the invention is to be restricted only in accordance with the appended claims.

I claim:

1. A method of treating an asphaltic stock comprising subjecting the stock to an elevated temperature in the presence of about 0.1 to 5.0% by weight of a fluoborate of a metal having an atomic number in excess of 22 and having a pronounced metallic character to decrease the temperature susceptibility of the stock.
2. A method of treating an asphaltic stock comprising heating and oxidizing the stock in the presence of about 0.1 to 5.0% by weight of a fluoborate of a metal having an atomic number in excess of 22 and having a pronounced metallic character to decrease the temperature susceptibility of the stock.

3. A method of treating pipe still bottoms comprising heating said material to about 200-300° F., adding about 1.0 to 3.0% by weight of a fluoborate of a metal having an atomic number in excess of 22 and having a pronounced metallic character, heating the mixture to about 425-450° F. and oxidizing said material to reduce the penetration to the desired value and to decrease the temperature susceptibility of the material.

4. A method of treating pipe still bottoms comprising heating said material to about 200-300° F., adding about 1.0 to 3.0% by weight of a fluoborate of a metal having an atomic number in excess of 22 and having a pronounced metallic character, maintaining the mixture

5 at a temperature of about 200-300° F. until visible evidence of reaction disappears, heating the mixture to about 425-450° F. and oxidizing said material to reduce the penetration to the desired value and to decrease the temperature susceptibility of the material.

## References Cited in the file of this patent

## UNITED STATES PATENTS

|           |                     |               |
|-----------|---------------------|---------------|
| 2,179,208 | Burk et al. _____   | Nov. 7, 1939  |
| 2,287,511 | Burk et al. _____   | June 23, 1942 |
| 2,494,510 | Hughes et al. _____ | Jan. 10, 1950 |
| 2,661,323 | Kraft _____         | Dec. 1, 1953  |